

# UNITED STATES PATENT OFFICE.

HORACE M. MURRAY, OF SELIGMAN, MISSOURI, ASSIGNOR TO J. W. DODGEN, OF OAK-GROVE, ARKANSAS.

## TANNING COMPOUND.

No. 869,723.

Specification of Letters Patent.

Patented Oct. 29, 1907.

Application filed January 7, 1905. Serial No. 240,079. Renewed May 3, 1907. Serial No. 371,661.

*To all whom it may concern:*

Be it known that I, HORACE M. MURRAY, a citizen of the United States, residing at Seligman, in the county of Barry and State of Missouri, have invented certain 5 new and useful Improvements in Tanning Compounds, of which the following is a specification.

This invention has for its object to provide a novel compound for coloring and tanning skins and hide.

The compound comprises, essentially, terra japonica, 10 fluid extract of crane's bill, alum and a coloring material, the latter for hides being preferably gum gambier. The proportions of the ingredients will vary according to the nature and age of the hide or skin and the length of time the same is to remain in the bath. The following proportions are given for approximately five gallons of water in the preparation of a bath for one to two 15 year old calf hides:

|                                 |        |
|---------------------------------|--------|
| Terra japonica.....             | 2 lbs. |
| Gum gambier.....                | 2 "    |
| Alum .....                      | 1½ "   |
| Fluid extract crane's bill..... | 1½ oz. |

The ingredients are mixed and the hide after being limed, depilated and bated, is immersed in the solution the required time until thoroughly tanned. For skins and small hides, the proportions will be less and 25 for cow, ox and horse hides the proportions will be increased. For example, the skin of a yearling is adapted to be readily tanned in a comparatively weak tanning solution, whereas the hide of a bull requires a longer time and a tanning solution of greater strength. 30 By varying the proportions of the ingredients to a given amount of water, the strength of the solution may be regulated to suit the nature of the hide to be tanned.

Having thus described the invention, what is claimed as new is:

A tanning solution consisting of water, gum gambier, terra japonica, alum, and crane's bill in about the proportions specified.

In testimony whereof I affix my signature in presence of two witnesses.

HORACE M. MURRAY. [L. S.]

Witnesses:

H. M. WALLACE,  
J. Z. SEXTON.